# EUROPEAN PATENT APPLICATION

(11) **EP 1 681 388 A2**
(43) Date of publication of application: **19.07.2006**
(21) Application number: 06447006.5
(22) Date of filing: 11.01.2006
(51) Int. Cl.: D06N 7/00, B44C 3/04

(54) **Floor covering having a jacquard fabric appearance**

(30) Priority: 12.01.2005 BE 200500016
(71) Applicant: Domo NV, 9052 Zwijnaarde (BE)
(72) Inventor: De Clerck, Jan, 9250 Waasmunster (BE)
(74) Representative: Brants, Johan P.E.

(57) **Abstract**

The present invention concerns a floor covering and a method for producing the same. The floor covering (1) comprises in particular a basic fabric provided with a projecting line pattern of at least two parallel lines (10) in at least two different directions. In particular, the floor covering is characterized in that 40 to 60 % of the total surface of the basic fabric comprises of inhibiting components, which are capable of forming a relief with the shape of said line pattern on the basic fabric.

## Description

### Technical field

The present invention concerns a decorative floor covering and a method for producing the same. As a special feature, the floor covering imitates a weave pattern, in particular a jacquard pattern, that is obtained by a specific pattern in relief using inhibition.

### Background of the invention

Jacquard fabrics already exist for many years in the textile sector. Jacquard fabrics are traditionally woven on jacquard looms to form detailed weave patterns. These patterns are characterized by fine lines or binding lines that extend in selective directions of the fabric. Despite its image of luxury and its high cost price, weaving jacquard fabrics has a lot of success in the decorative sector. The jacquard weaving technique is applied among others in the production of furniture fabrics, curtains, etc. The rich look of jacquard-chenille fabrics is characterized by its 2-3 dimensional effects and the relief caused by the type of yarn used and the binding and/or the fine lines formed. The jacquard fabrics may exhibit a rich and luxurious look.

However, jacquard fabrics are not inexpensive to produce. Hence, in the prior art procedures were developed to imitate jacquard fabrics. For example, US patent US 5,685,223 describes a technique to imitate a jacquard motif on a fabric and to reproduce three-dimensional patterns on a fabric by using printing techniques. However, the process described is not suited to be applied for imitating a jacquard motif on a synthetic covering, such as, for example, a floor, wall or ceiling covering.

Techniques for printing of synthetic coverings in order to obtain patterns in relief are also known in the prior art. These techniques differ among others on the inks used and the manner to obtain the patterns in relief. For example, the European patent application EP 0 449 012 refers to a method for manufacturing a synthetic material which obtains a 3D motif using a printing technique. The decorative material described in EP 0 449 012 consists of a basic material upon which a printing pattern is applied showing a relief. The printing pattern is formed by a composition consisting of the reaction of a PVC resin and a reactive acrylic resin. The PVC resin provides for the preservation of the relief, while the acrylic resin induces a curing. The acrylic resin in the composition is activated by means of ionising radiation, peroxide or heat.

The US patent US 3,905,849 describes a floor or wall covering exhibiting a relief. The covering consists of a transparent (PVC, PE, polyester) layer which is provided on the bottom side with a) a decorative layer, b) one or more intermediate layers consisting of a paste, and c) a supporting layer. By impressing during the laminating process, the paste applied on the bottom side of the covering will induce a pattern in relief towards the top side of the covering.

The European patent 0 003 965 describes a polymer material used for the manufacturing of a decorative product. The material comprises essentially three layers : a foamable substrate, on which an intermediate layer is applied that forms a design or pattern on the substrate, and finally a surface coating of a resin-like, polymer material. In the intermediate layer reactive polymerisable monomers are present, as is also a polymerisation initiator, which is provided on specific locations distributed over the intermediate layer. This initiator is capable of inducing cross-linking and polymerisation of said monomers. Upon heating the top surface coating, the underlying substrate is foamed, while in the intermediate layer polymerisation is induced near the initiator. Therefore, in the surface coating the melt viscosity is increased locally, and more specifically in those areas that cover the intermediate layer with initiator, such that a pattern in relief is created.

However, the techniques described above have the drawback that they do not provide the printed and/or heat-treated materials with the look of a jacquard fabric.

Therefore, the goal of the present invention is to provide a synthetic material on which a jacquard motif has been imitated. More particularly, the goal of the invention is to provide a synthetic covering which has the look of a jacquard fabric.

The goal of the present invention is also to provide a simplified and efficient method for the manufacturing of a synthetic covering having the look of a jacquard fabric.

### Summary

The present invention provides in a first aspect a floor covering comprising a basic fabric provided with a projecting line pattern of at least two parallel lines in at least two different directions, characterized in that 40 to 60 % of the total surface of the basic fabric consists of inhibiting components, which are capable of producing on the basic fabric a relief with the shape of said line pattern.

The jacquard-chenille designs on the basic fabric are preferably composed of geometrical patterns, and in particular of different line motifs. These line motifs have different of equal dimensions (length-width) and may consist of one of more colours, and may be positioned in at least two different directions and degrees of angle. By these combinations weaves and/or fine lines of the jacquard-chenille technique are simulated and a 2-dimensional image is obtained. By the production process, this 2D-image becomes three-dimensional. The 3D-effect arises from the following factors : the engraving of geometrical patterns/line motifs in at least two different directions in one or more colours, the use of inhibitor in these engraved motifs, such that no foaming is produced relative to the background layers provided on the basic fabric. Hence, different differences in height arise wherein a structure in relief is created and mechanical embossing is simulated. The reflection of the light on the covering also provides for the creation of different degrees of sheen and colour differences, such that also optically different motifs are created.

In a second aspect, the present invention provides a method for manufacturing a floor covering consisting of a carrier having different layers mainly consisting of plastisol applied thereon. The method comprises the subsequent steps of:
a) providing a carrier,
b) applying and curing a non-foamable basic layer on one side of the carrier from a),
c) applying and curing a foamable top foam layer on the basic layer applied in b),
d) applying a line motif on the top foam layer applied in c) using an engraving process,
e) applying and curing a foamable backing layer on the bottom side of the carrier, and
f) applying a surface coating on the top foam layer applied in e), and
g) foaming the whole of layers obtained in f) in order to obtain a floor covering.

To the printing ink that is (are) used in step d) of the process, inhibitor may be added which is also printed on the top foam layer and acts on that layer. In a preferred embodiment, the method provides the use of 20 to 40 % of inhibitor in the printing ink that is used to print the top foam layer. Optionally, the covering obtained in f) may further be provided with a layer of varnish. The backing layer may be foamed by means of a mechanical or chemical process.

In order to better demonstrate the features of the invention, hereafter, a few preferred embodiments of a covering according to the present invention are described as an example, without being limited thereto.

### Description of the figures

Figure 1 is a schematically exploded view of an embodiment of a covering according to the present invention.
Figure 2 depicts a top view of an embodiment of a covering according to the present invention showing the line pattern.

### Detailed description

The present invention concerns a covering having the look of a jacquard fabric. Hereafter, the invention will be described in particular with reference to a floor covering. It is obvious that the present invention may also concern a synthetic material with the look of a jacquard fabric that may be used for other purposes, such as for example a wall covering, ceiling covering, table or desk covering, car lining, and the like.

In a first embodiment the invention provides a floor covering comprising a basic fabric which is provided with a projecting line pattern of at least two parallel lines in at least two different directions. The covering is in particular characterized in that 40 to 60 %, and for example 45, 47, 50, 52, 55 or 57 % of the total surface of the basic fabric consists of inhibiting components. These inhibiting components are capable of producing a relief with the shape of said line pattern on the basic fabric.

Preferably the inhibiting components comprise thiourea or benzotriazol.

In another embodiment, the invention provides a covering, characterized in that at least 40 % of the total surface of the basic fabric, and for example 45 %, 50 %, 55 %, 60 %, 65 % or 70 % of the total surface of the basic fabric, is provided with a line pattern of at least four, and preferably of at least six, seven or eight parallel lines in at least two different directions.

In a particularly preferred embodiment, said two different directions comprise perpendicular directions, and preferably an horizontal and a vertical direction. It is obvious that said line pattern may also be provided in more than two directions, and for example in an horizontal, vertical and inclined direction.

The present invention provides a covering, characterized in that said lines have a height which ranges between 0.15 and 0.35 mm.

In a further embodiment, the invention provides a covering, characterized in that said lines have a thickness which ranges between 1.0 and 2.0 mm.

In yet another embodiment, the invention provides a covering, characterized in that said lines have a mutual distance which ranges between 1.0 and 2.0 mm.

The invention also concerns a covering characterized in that the basic fabric has a thickness which ranges between 0.20 and 0.50 mm.

The invention further provides a covering characterized in that the ratio between the number of lines in one direction and the number of lines in another, preferably perpendicular direction ranges between 40:60 and 60:40, and amounts for example 45:55, 48:52, 50:50, 52:48 or 55:45.

On the basic fabric, so-called "islands" may be distinguished. The term "islands" refers to surfaces on the basic fabric which are formed by at least four parallel lines. The line motif on the basic fabric is formed from a combination of smaller surfaces (=islands) where the lines run in parallel. Depending on the direction of the parallel lines, different "islands of direction" may be distinguished. A "vertical island of direction" refers to an island formed by at least four lines which run parallel in a vertical direction. An "horizontal island of direction" refers to an island formed by at least four lines which run parallel in an horizontal direction. It is obvious that also other islands of direction are possible, depending on the direction in which the parallel lines are running. At least two types of islands of direction may be present, and preferably perpendicular relative to each other if there are effectively only two.

In a preferred embodiment, the invention provides a covering, characterized in that the basic fabric is provided with islands formed by at least four parallel lines, and of which at least 50 %, and preferably at least 60 %, at least 70 %, at least 80 %, and more preferably even at least 85 % are larger than 10 cm², and preferably larger than 15 cm², and more preferably even larger than 20 cm².

In another preferred embodiment, the invention provides a covering, characterized in that at least ten, and preferably at least twenty, and more preferably at least thirty different islands are provided per m² of basic fabric.

Preferably, the invention provides a covering in which the basic fabric is provided with at least two different islands of direction, for example a vertical and a horizontal island of direction.

ln a preferred embodiment, the invention provides a covering, characterized in that the basic fabric is provided with at least ten, and preferably at least twenty, vertical islands of direction per m² of basic fabric. In yet another preferred embodiment, the invention provides a covering, characterized in that the basic fabric is provided with at least ten, and preferably at least twenty, horizontal islands of direction per m² of basic fabric. The invention further provides a covering, characterized in that the ratio between two different islands of direction, for example the ratio between a vertical and an horizontal island of direction, ranges between 40:60 and 60:40, and amounts for example 45:55, 48:52, 50:50, 52:48, or 55:45.

In yet another embodiment the invention provides a covering, characterized in that one of more designs are superimposed upon the basic fabric. Such a superimposed design is left open in the basic fabric or line motif-design. More particularly, the invention provides a covering in which at most 20 %, and preferably at most 15 %, and more preferably even at most 10 % of the basic fabric is further provided with one or more designs, which are superimposed on the basic fabric. Preferably, 60 % to 80 %, and for example 65 %, 67.5 %, 70 %, 72.5 %, 75 % or 77.5 % of the surface of each design is provided with lines in one direction. The superimposed design is preferably uniformly distributed over the basic fabric. This design may optionally be inhibited or coloured.

The present floor covering may have one colour (monochrome) or many colours (polychrome). For example, the basic fabric may have one colour. In another example, different colours may be provided in the basic fabric. Similarly, the superimposed design may have one colour or may have more colours. In yet another example, the basic fabric and the design may have one colour but they may have a mutually different colour. In yet another example, both basic fabric and design may have many colours.

The basic fabric of a covering according to the present invention consists preferably of a carrier provided at the top with a non-foamable basic layer and a foamable top foam layer applied thereon (weight 200-400 g/m², and for example 280 g/m²). For example, the carrier may be a fibreglass sheet carrier. Preferably, the carrier has a weight of 40 g/m² and for example has a thickness of for example 0.35 mm.

The basic fabric may be further provided on top and bottom side with a number of extra layers. In an embodiment, the invention provides a covering, characterized in that a foamable backing layer is provided on the back of the basic fabric.

In another embodiment, the covering may further be provided with a transparent surface coating, applied on top of the basic fabric. Preferably, the surface coating has a specific gravity of 220 - 440 g/m² and for example 250 g/m².

Optionally, a layer of varnish may further be applied on this surface coating. This layer of varnish consists preferably of polyurethane, and preferably has a thickness of 12 ± 5 µm. This layer of varnish preferably comprises a PU-dispersion on a water basis which yields an improved resistance against staining and abrasion resistance, after drying and curing with UV-light, and which allows the modification of the degree of sheen of the covering.

Preferably, the present floor covering has a total thickness which ranges between 0.50 and 5 mm.

According to a more particularly preferred embodiment, the present invention provides a covering comprising a carrier, and a number of layers of plastisol applied thereon, also called polymeric pastes. The term "plastisol" as used herein, refers to a paste composition comprising a polymer, such as for example, but not limited to, PVC, polyethylene, polypropylene, polyurethane, and the like, and preferably PVC.

Every plastisol layer shows specific properties and is manufactured using a specific paste composition. These pastes are liquid and highly viscous at room temperature, but jellify (= cure) quickly at ± 140 °C. Such a paste preferably is a mixture of one or more of the following components :
- a suitable polymer, preferably PVC powder
- a filler, for example chalk,
- plasticizers,
- additives, such as, for example, thermostabilisers, bleeders, viscosity regulators, and the like,
- a foam-producing agent (foaming batch), such as, for example, azodicarbonamide and the like. This foam-producing agent is pre-formulated for dosing in the plastisol and is used in those specific product layers that require foaming. Certain molecules such as, for example, azodicarbonamide, that are latently present at room temperature in these specific plastisols, will decompose at higher temperatures of ± 180°C and higher, into small gaseous molecules, such that in this decomposition reaction a large gas volume is released that settles with the shape of small regular-shaped gas bubbles in the plastisol matrix. In combination with the simultaneously running curing process, in this manner a foam structure is created.

Preferably, different pastes are provided for different plastisol layers. In an example, the basic layer, which serves as levelling layer for covering of the fibreglass sheet carrier, consists mainly of a polymer such as, for example, PVC, PE, PU, and a filler, preferably chalk.

In another example, the foamable top foam layer consists mainly of a mixture of a polymer such as, for example, PVC, PE, PU, a filler, preferably chalk, a foaming agent, preferably azodicarbonamide, and 20 to 40 % of inhibitor, preferably thiourea or benzotriazol.

Preferably, the covering is further provided with a foamable backing layer applied on the back of the basic fabric. This backing layer may be both chemically foamable or mechanically foamable. A chemically foamable backing layer refers to a layer formed by a paste comprising a foaming agent, such as defined above. In the paste formula of mechanical backing foam, no foaming agents are present. With a very performative mixer (mondomixer), supplied air is divided very finely in tiny air bubbles and whipped as such into the paste. This air is well trapped into the paste matrix by a soap component that was added to the paste. At higher temperatures, only curing of the foam occurs, and no chemical reaction is needed.

The surface coating of the covering, also called wear-resistant layer, that is applied on top of the printed line motif, is a transparent layer (and hence contains no fillers).

Referring to figure 1, an embodiment of a covering according to the present invention is schematically depicted. The covering 1 consists of a substrate 2 comprising a fibreglass sheet carrier 3, impregnated with a basic layer (not shown), and a top foam layer 4 applied thereon. At the bottom side of the basic fabric, a backing foam layer 5 is provided. On top of the basic fabric, a transparent surface coating 6 may be applied. The whole is further finished by applying a transparent layer of varnish 7 on the surface coating.

Referring to figure 2, a top view of a covering according to the present invention is depicted. The covering comprises a basic fabric provided with a projecting line pattern of at least two parallel lines 10 in vertical and horizontal direction. On the covering, vertical islands of direction 8 and horizontal islands of direction 9 may be distinguished. These comprise surfaces which are formed by at least four parallel lines 10. Further, multiple designs 11 were also applied on the covering.

### Examples

Examples 1 and 2 illustrate methods for manufacturing coverings according to the present invention.

### Example 1

### Step 1 : Unroller = starting point of the production.

Carrier material is unrolled. Different types of carrier may be used, but preferably, a fibreglass carrier is used.

### Step 2 : Ironing work 1.

This step comprises applying and levelling a first layer of paste on the carrier. This first layer is highly filled with chalk and is 100 % compact (hence, no foaming agents are latently present). This basic layer is led over a chromium-plated and heated (140 ± 10°C) jellifying drum, wherein the paste is levelled and cured. Subsequently, the fabric is led over cooling rollers and cooled.

### Step 3 : Ironing work 2.

In this step, a second layer of paste is applied, the top foam. Herein, the molecules are latently present which later in the production process will foam. This layer is cured in an oven (160±10 °C), but is not foamed yet.

### Step 4 : Pressure hall.

This step comprises applying a line motif using the engraving procedure on the top foam layer, i.e. different pressure rollers each printing a part of the motif with a specific colour on the fabric. It is obvious that the whole of rollers should be positioned very precisely relative to each other (= repeated). Inhibitor may be added to one or more of the printing inks used. These are molecules that locally, only where the inhibitor is printed, impede the foaming process of the underlying foam layer. In fact, they act upon the "kicker" (preferably zinc oxide or a zinc oxide containing composition) which acts as a catalyst for the foaming process. The action of this "kicker" is stopped by an inhibitor (preferably thiourea or benzotriazol), such that the foaming process is locally stopped and hence, a relief is created.

### Step 5 : Ironing work 3.

This step comprised applying a layer of paste on the back (bottom side) of the sheet fabric. This layer of paste is called backing foam, hence foaming agents are latently present which further onwards in the production process will provide for foaming of the product. At first instance, this layer is only cured on a jellifying drum (140 + 10°C). This backing foam will determine the final thickness of the floor covering. This manner of working yields products with a final thickness of preferably 2 mm. For thicker floor coverings, in this step also a backing foam is applied, but this happens later (see below - example 2).

### Step 6 : Ironing work 4.

This step comprises applying the surface coating (wear-resistant layer). This is a transparent layer (hence, contains no fillers) that is applied on top of the printed line motif. It is cured in an oven in which temperatures rise up to 200 ± 10°C and hence, in which also all foaming agents latently present in one or two layers, react and foam the product, except on those places that are printed with inhibitor, such that the product, when leaving this oven, also shows a relief structure.

### Step 9 : Final control and packaging.

In this step, the finished product is visually inspected for errors, packed and optionally stored.

### Example 2

This example illustrates the production of coverings with a thickness starting at 2 mm. According to this method, it is possible to differentiate with regard to the backing layer : it is possible to use chemical backing foam or mechanical backing foam. With the latter, no foaming agents are present in the paste formulation, as explained above.

### Step 1 : Unroller line = starting point of the production.

In this step, a product is unrolled which may be obtained according to example 1 but which has not been provided with a backing layer.

### Step 2 : Ironing work 5

This step comprises applying a mechanical or chemical backing layer. This backing layer is cured and/or foamed in an oven (temperatures up to 200 ± 10 °C). Weight depends entirely of the desired final thickness of the floor covering.

### Step 3 : Paint room.

Using the engraving procedure, a thin layer (12 ±5 µm) of polyurethane coating is applied onto the wear-resistant layer.

### Step 4 : Imprinting.

In this step, the wear-resistant layer is reheated and softened (160 ± 10 °C) after which the fabric is pressed between a water cooled imprinting roller and a rubber counter roller. The imprinting roller is a steal roller with an engraved relief structure that is transferred at high pressure and temperature to the fabric. The cooling, as it were, freezes the relief structure in the fabric.

### Step 9 : Final control and packaging.

The product is now finished : it is now visually inspected for errors, packed and send to the warehouse for storage.

### Example 3

In an example, a floor covering according to the present invention consists of:
- fibreglass sheet: 0.35 mm, 40 g/m²
- basic layer: 550 g/m²
- top foam : 280 g/m²
- surface coating : ranging between 0.20 and 0.40 mm
- backing foam : mechanical backing foam, thickness arbitrarily up to 4.0 mm.

## Claims

1. Floor covering (1) comprising a basic fabric provided with a projecting line pattern of at least two parallel lines (10) in at least two different directions, **characterized in that** 40 to 60 % of the total surface of the basic fabric consists of inhibiting components, which are capable of producing on the basic fabric a relief with the shape of said line pattern.

2. Covering according to claim 1, **characterized in that** at least 40 % of the total surface of the basic fabric is provided with a line pattern of at least four, and preferably at least six to eight parallel lines in at least two different directions.

3. Covering according to claim 1 or 2, **characterized in that** said two different directions are perpendicular directions.

4. Covering according to one of the preceding claims 1 to 3, **characterized in that** said lines have a height which ranges between 0.15 and 0.35 mm.

5. Covering according to one of the preceding claims 1 to 4, **characterized in that** said lines have a thickness which ranges between 1.0 and 2.0 mm.

6. Covering according to one of the preceding claims 1 to 5, **characterized in that** said lines have a mutual distance which ranges between 1.0 and 2.0 mm.

7. Covering according to one of the preceding claims 1 to 6, **characterized in that** the ratio between the number of lines in one direction and the number of lines in another, preferably perpendicular direction ranges between 40:60 and 60:40, and amounts for example 50:50.

8. Covering according to one of the preceding claims 1 to 7, **characterized in that** the basic fabric has a thickness which ranges between 0.20 and 0.50 mm.

9. Covering according to one of the preceding claims 1 to 8, **characterized in that** the basic fabric is provided with islands (8, 9) formed by at least four parallel lines, of which at least 50 %, and preferably at least 80 % is larger than 10 cm².

10. Covering according to preceding claim 9, **characterized in that** at least ten, and preferably at least twenty different islands are provided per m² of basic fabric.

11. Covering according to preceding claim 9 or 10, **characterized in that** the basic fabric is provided with at least two different islands of direction, for example a vertical (8) and an horizontal island of direction (9).

12. Covering according to one of the preceding claims 9 to 11, **characterized in that** the ratio between two different islands of direction, for example the ratio between a vertical and an horizontal island of direction ranges between 40:60 and 60:40.

13. Covering according to one of the preceding claims 1 to 12, **characterized in that** at most 20 % of the basic fabric is further provided with one or more designs (11), which are superimposed upon the basic fabric.

14. Covering according to claim 13, **characterized in that** 60 to 80 % of the surface of each design is provided with lines in one direction.

15. Covering according to one of the preceding claims 1 to 14, **characterized in that** the basic fabric consists of a carrier (3) which is provided on top with a non-foamable basic layer and foamable top foam layer (4) applied thereon.

16. Covering according to one of the preceding claims 1 to 15, **characterized in that** the covering is further provided with a foamable backing layer (5) that is applied on the back of the basic fabric.

17. Covering according to one of the preceding claims 1 to 16, **characterized in that** the covering is further provided with a transparent surface coating (6) that is applied on top of the basic fabric.

18. Covering according to one of the preceding claims 1 to 17, **characterized in that** the covering is further provided with a layer of varnish (7) that is provided on the surface coating of the basic fabric.

19. Covering according to one of the preceding claims 1 to 18, **characterized in that** the covering (1) has a total thickness which ranges between 0.50 and 5.0 mm.

20. Method for manufacturing a floor covering consisting of a carrier having different layers of plastisol applied thereon, comprising the steps of:
a) providing a carrier (3),
b) applying and curing a non-foamable basic layer on one side of the carrier from a),
c) applying and curing a foamable top foam layer (4) on the basic layer applied in b),
d) applying a line motif on the top foam layer applied in c) using an engraving process,
e) applying and curing a foamable backing layer (5) on the bottom side of the carrier,
f) applying a surface coating (6) on the top foam layer obtained in d), and
g) foaming the whole of layers obtained in f) in order to obtain a floor covering.

21. Method according to claim 20, wherein foaming occurs in g) by heating to a temperature of 200° ± 10 °C.

22. Method according to claim 20 or 21, wherein 20 to 40 % of inhibitor is used in the printing ink used to print the top foam layer (4).

23. Method according to one of the preceding claims 20 to 22, wherein the backing layer (5) is foamed using a mechanical or chemical process.

24. Method according to one of the preceding claims 20 to 23, wherein the covering obtained in g) is further provided with a layer of varnish (7).
